

Aug. 25, 1925.

1,551,192

F. G. FEILER

LAMINATED FABRIC FOR SCOURING DEVICES, ETC

Filed Sept. 8, 1922

*Fig. 1*



*Fig. 2*



Inventor

Fred G. Feiler  
By his Attorneys  
Emory Farney, Blair & Bogart.

Patented Aug. 25, 1925.

1,551,192

# UNITED STATES PATENT OFFICE.

FRED G. FEILER, OF IRVINGTON, NEW JERSEY, ASSIGNOR TO SAMUEL J. BRAUN, OF SYRACUSE, NEW YORK.

## LAMINATED FABRIC FOR SCOURING DEVICES, ETC.

Application filed September 8, 1922. Serial No. 587,011.

*To all whom it may concern:*

Be it known that I, FRED G. FEILER, a citizen of the United States, and a resident of Irvington, county of Essex, State of New Jersey, have invented an Improvement in Laminated Fabrics for Scouring Devices, Etc., of which the following is a specification.

The present invention relates to metal 10 wool fabrics adapted for use for scouring devices and for other uses.

The principal object of the invention is to provide an improved fabric, combining steel wool or its equivalent with other 15 fibrous material, which is adapted for use for scouring and for other uses.

Steel wool has been used for scouring aluminum or other kitchen ware, but when used by itself it is unpleasant to hold in the 20 hand because of its rough and prickly nature, and it is objectionable because short lengths of the fibre break off and work loose from the mass. Steel wool alone is 25 unsatisfactory for some uses because it will not retain soap or water to any substantial extent and must be used either practically dry or must be frequently moistened.

The present invention provides an improved arrangement in which the fibrous 30 material is combined with metal wool in such a way that it serves to form a support or binding for the metal fibres and a projection for the hand. The combination with the metal wool of cotton or other fibre 35 of a suitable nature serves also to retain both soap and water so that the scouring can be done as a wet operation.

The nature and object of the invention 40 will be better understood from a description of a particular illustrative embodiment thereof, reference being had to the accompanying drawings, in which

Figure 1 is a perspective view of a section 45 of material constructed in accordance with the invention;

Figure 2 is a sectional view of the same, illustrating the manner in which the fibres of the cotton or similar material and the metal wool are extended through the mass 50 to hold the same together.

The particular embodiment shown in the drawings, for the purpose of illustrating the principles of the invention, is a scouring pad having steel wool combined with fibrous material. As shown, the steel wool is in the

form of a relatively thin layer 5 and is combined with a layer 6 of vegetable fibre or equivalent material in such a way that the two are united rather firmly to each other. The fibre may be of a character to retain 60 soap and water to facilitate wet scouring and is preferably loosely matted and so united to the steel wool that it serves at least partially to protect the hands of the user. Preferably the opposite side of the 65 metal is protected by a fibrous binder as, for example, a loosely woven fabric 7.

The three parts of the pad are suitably secured together. This is preferably done by interengaging the fibres of the parts to 70 form a bond therebetween. In the structure illustrated a number of fibres of the protective layer 6 extend into or through the metal layer and preferably even through the fabric layer 7 as indicated at 8. Similarly threads of the steel wool extend through the fabric and form a bond between the steel wool and the fabric, as indicated at 9. This arrangement of the metal fibres 75 accomplishes two purposes; it binds together the metal and fabric and it causes the abrasive metal fibres to be presented upon the outer side of the fabric to provide an operative abrasive surface. In use other fibres of the metal wool gradually work 80 through the fabric 7 and thus maintain the abrasive surface.

The described arrangement is produced effectively by arranging the material in layers as shown and then by forcing forked 90 needles through the material from the fibre side, (i. e. upwardly in the drawing). The fibres of the layer 6 and also the fibres of the metal wool 5 are thus pushed through the mass and through the fabric 7 at substantially a right angle to the plane of the material. This method of securing the metal to the fabric presents apparent difficulties, due to the nature of the metal operated upon, but it has been found in practice that 100 a sufficient number of fibres of the metal can be bent and forced through the fabric to form the desired bond without breaking the same. The operation also brings to the free side of the fabric 7 a sufficient number 105 of metal fibres to provide the desired scouring surface.

Some of the needles as pushed through will generally engage both vegetable and mineral fibres, which together pass through 110

the fabric and form a more effective bond than either the vegetable or the mineral fibres could alone effect.

The bond formed between the metal and the fabric by the metal fibres which are forced through the fabric is sufficiently effective to hold the metal and fabric in a substantially permanent sheet even if the vegetable fibre 6 is omitted as is desired 10 when the material is used for some purposes other than scouring.

The fabric 7 may be omitted if the purposes for which the material is to be used are such that the fibre and metal wool will 15 form a sufficiently durable sheet, and if the retention of the loose broken metal fibres by the fabric is not desired.

The material described can be easily manufactured with inexpensive machinery, since 20 sheets of felted steel wool as well as felted fibre can be purchased as articles of commerce. It is to be noted that the manner of punching the fibres through the mass described leaves one side of the mass substantially free of any metal and reasonably 25 smooth, while the other side presents an effective abrasive surface.

This specification defines the described material more particularly with regard to 30 the one use mentioned, but the invention con-

templates other uses of the material where metal wool in sheet form combined with a binder or protective surface of the character described is of value, and obviously the material is capable of numerous uses 35 not herein mentioned.

I claim as my invention:

1. A scouring device of the character described comprising a layer of metal wool scouring material, a protective layer of fibrous material on one side and a loosely woven fabric binder on the other side of said metal wool, fibres of the metal wool extending in loops through the fabric binder and fibres of the protective layer extending in loops through both the metal wool and the fabric binder to secure together the respective parts substantially as and for the purpose described.

2. A device of the character described comprising a layer of metal wool, a protective layer of fibrous material on one side thereof, fibres of one material extending transversely through the layer of the other material to form a binder between the two 55 materials.

In testimony whereof, I have signed my name to this specification March, 1922.

FRED G. FEILER.